

## UNITED STATES PATENT OFFICE

1,921,148

YEING AND PRINTING OF TEXTILE FIBERS  
BY MEANS OF DYES FORMED BY OXIDA-  
TIONMartin Battegay, Mulhouse, France, assignor to  
Calco Chemical Company, Inc., a Corporation  
of New JerseyNo Drawing. Application August 13, 1930  
Serial No. 475,116

20 Claims. (Cl. 8—5)

My invention relates particularly to a process of dyeing and printing of fibres by means of dyes formed by oxidation and relates to the dyeing of fibers or fabrics of any desired character.

- 5 The object of my invention is to provide an improved process of the above character in which dyeing may be carried out in an advantageous manner by use of the materials as hereinafter referred to. In my previous application upon  
10 Process for the preparation of sulfocyanate complex paraphenylenediamine and similar amines, Ser. No. 399,392, filed October 12, 1929, I have described the preparation of a complex sulfocyanate of paraphenylenediamine and the application of the same in dyeing. As an improvement over the same I have discovered that the dyeing and printing of fibers, particularly textile fibers of any desired kind, as for example, cotton, may be advantageously carried out by means of dyes  
15 formed by oxidation of products, which are characterized as transformation products of sulfocyanates and their homologous derivatives or substitution products, as well as similar products in the dyeing and printing operations, capable of being used either alone or in combination with the usual colors formed by oxidation. See Lellmann (Liebigs' Annal, vol. 221, page 11, (1883)), Frerichs and Hupka. (Archiv der Pharma., vol. 241, page 162, and Beilstein (1930), Vol. XIII, page 105). Of the most practical products I may mention among the products of transformation of the sulfocyanates, for instance, the phenylenedithioureas and the monoaminophenylthioureas; and then among the homologous derivatives or substitution products, the toluylene ditioureas and the monoaminotolylthioureas; and finally, among the similar products, for instance, the compounds resulting from the condensation of aldehyde or ketone bisulfite addition products with amines, such as the sodium salt of methylaminophenyl- $\omega$ -sulfonic acid, and the sodium salts of the methylaminotolyl- $\omega$ -sulfonic acids, the sodium salts of the monomethylphenylenediamine- $\omega$ -sulfonic acids, and the sodium salts of the phenyl-monomethylphenylenediamine- $\omega$ -sulfonic acids, etc.

As pointed out above, these products are capable of being used in place of the products mentioned in the above application for Letters Patent in combination with the usual dyes formed by oxidation or alone to secure the same type of dyeing with the aid of oxidation. When used in the place of the product referred to in the above application for Letters Patent, these products

used in accordance with the present application can be directly incorporated in the dye solutions or printing pastes of the dyes of the usual type made by oxidation in order to apply them to the fibrous materials, or if desired, they can be applied separately to said materials by having them preceded or followed by the usual oxidized dyes.

While my invention is capable of being carried out in many different ways, for the purpose of illustration I shall now describe certain examples of the same:

## 1st example for the preparation of the dye bath

|                                                                                                                                                                                                                                                               |    |
|---------------------------------------------------------------------------------------------------------------------------------------------------------------------------------------------------------------------------------------------------------------|----|
| 75 gms. an aniline salt                                                                                                                                                                                                                                       | 70 |
| 150 cc. water                                                                                                                                                                                                                                                 |    |
| 30 gms. sodium chlorate                                                                                                                                                                                                                                       |    |
| 150 cc. water                                                                                                                                                                                                                                                 |    |
| 3 to 8 gms. of phenylenedithiourea, or the equivalent quantity of mono-aminophenylthiourea, or the sodium salt of mono-methylphenylenediamine- $\omega$ -sulfonic acid, or the sodium salt of phenylmono-methylphenylenediamine- $\omega$ -sulfonic acid, and | 75 |
| 100 cc. of 20% acetic acid                                                                                                                                                                                                                                    |    |
| 60 gms. sodium ferrocyanide dissolved in 150 cc. water                                                                                                                                                                                                        |    |

The whole being diluted if desired to 1 liter of solution. 85

## 2nd example for the preparation of the dye bath

|                            |    |
|----------------------------|----|
| 75 gms. of aniline salt    |    |
| 150 cc. of water           |    |
| 30 gms. of sodium chlorate | 90 |
| 150 cc. water              |    |

|                                                                                                                                                                                                                                                |    |
|------------------------------------------------------------------------------------------------------------------------------------------------------------------------------------------------------------------------------------------------|----|
| 3 to 8 gms. of phenylenedithiourea, or the equivalent quantity of mono-aminophenylthiourea, or the sodium salt of mono-methylphenylenediamine-sulfonic acid, or the sodium salt of phenylmonomethylphenylenediamine - $\omega$ - sulfonic acid | 95 |
| 100 cc. of 20% acetic acid, and                                                                                                                                                                                                                |    |
| 8 cc. of ammonium vanadate (1: 1000)                                                                                                                                                                                                           |    |

The whole, if desired, in the above example may be diluted to one liter by adding water. 100

For dyeing, in accordance with these examples, the textile fiber is impregnated with one of the preceding preparations, then centrifuged or pressed, and dried at a temperature not above 55° C. The color is developed either by a short usual steaming or by a prolonged airing, such as is customary for the development of oxidized colors. The dyed fiber is afterward passed through a dilute sodium carbonate bath comprising 110

ing water containing 5% by weight of sodium carbonate to which has been added, if need be, the usual quantity of an alkaline chromate, that is to say,—

5 1000 cc. of the sodium carbonate solution  
10 gms. sodium chromate

By this method dyeings are effected by means of oxidized colors without damaging the textile fiber.

10 For printing it is preferable to use pastes containing the same proportions of the various constituents used in the two above mentioned examples by replacing any desired part of the water by a corresponding quantity of a suitable thickener. Such a thickener may be starch-tragacanth for instance. 3rd example for the preparation of the dye bath:

*A Solution "A" is prepared containing*

20 24 cc. aniline oil  
24 cc. 22° Bé. hydrochloric acid  
2 gms. of tartaric acid, and  
150 cc. of water

*A Solution "B" is made containing*

25 7 gms. of sodium chlorate  
5.5 gms. of copper sulfate  
5.5 gms. of ammonium chloride  
200 cc. of water

30 and finally Solution "C" containing 3 to 8 gms. of sodium monomethylphenylenediamine- $\omega$ -sulfonate, or of sodium phenylmonomethylphenylenediamine- $\omega$ -sulfonate, and  
100 cc. of water

35 The three solutions, A, B and C may be mixed just before being used and the operation is then carried out as under Examples 1 and 2.

The composition of this preparation can be equally well used for printing by proceeding as 40 mentioned above, on the one hand by replacing a part of the water by a suitable thickener, and on the other hand by replacing the copper sulfate by 5 gms. of an insoluble copper salt, such as copper sulfide, for instance.

45 In the case where the above mentioned products precipitate with copper salts, the impregnation is carried out in two operations by milling the textile, for instance, in a first operation with a solution of 3 to 8 gms. of monoamino-50 phenylthiourea dissolved in 40 cc. of 20% acetic acid and 960 cc. of water and then, after squeezing, passing in a mixture of Solutions A and B above mentioned.

To illustrate those of the above similar products which lend themselves to obtaining practical oxidized dyes, we will mention, for instance, the sodium salt of methylaminophenyl-sulfonic acid, or the sodium salt of methylaminoorthotolyl-sulfonic acid, which yield intense brown colors 60 by applying on the fiber, for instance, one of the following preparations:

*4th example for the preparation of the dye bath*

200 gms. of sodium methyl-aminophenyl- $\omega$ -sulfonate, or of sodium methyl-aminoortho-tolyl- $\omega$ -sulfonate

300 cc. water  
75 to 100 gms. of sodium chlorate  
20 gms. of ammonium chloride  
385 cc. water  
20 cc. of vanadyl chloride (1:1000)

*5th example for the preparation of a dye bath*

200 gms. of sodium methyl-aminophenyl- $\omega$ -sulfonate, or of sodium methylaminoortho-tolyl- $\omega$ -sulfonate

300 cc. water  
75 to 100 gms. of sodium chlorate  
20 gms. of ammonium chloride  
20 cc. of a 50% copper sulfate solution, and  
385 cc. water.

The application on the fiber may be carried out exactly under the same conditions as given in Examples 1, 2 and 3.

It can also be carried out according to the printing method by making the above mentioned modifications, for example as referred to under the 2nd example.

In the above examples the sodium chlorate acts as an oxidizing agent; the acetic acid, hydrochloric acid, and tartaric acid are provided to control the color desired and as solvents; the ammonium vanadate and the vanadyl chloride assist in the oxidation and act as catalysts; the copper sulfate acts as a catalyst and also assists in the oxidation.

While I have described my invention above in detail, it is to be understood that many changes may be made therein without departing from the spirit of the same as set forth in the claims.

I claim:

1. The process which comprises dyeing a fibrous material with the aid of a dyeing composition containing a member of a group of substances which consists of transformation products of sulfocyanate derivatives of the benzene series.

2. The process which comprises dyeing a fibrous material with the aid of a dyeing composition containing a phenylene dithiourea.

3. The process which comprises dyeing a fibrous material with the aid of a dyeing composition containing a dye formed by oxidation, and as another dye, a member of a group of substances which consists of transformation products of sulfocyanate derivatives of the benzene series.

4. The process which comprises dyeing a fibrous material with the aid of a dyeing composition containing a dye formed by oxidation, and as another dye, a phenylene dithiourea.

5. The process which comprises dyeing a fibrous material with the aid of a dyeing composition containing a dye formed by oxidation, and as another dye, a member of a group of substances which consists of transformation products of sulfocyanate derivatives of the benzene series, one of said dyes being applied first and the other dye being applied later to the fibrous material to be dyed.

6. The process which comprises dyeing a fibrous material with the aid of a dyeing composition containing a dye formed by oxidation, and as another dye, a member of a group of substances which consists of transformation products of sulfocyanates of the benzene series, one of said dyes being applied first and the other dye being applied later to the fibrous material to be dyed.

7. The process which comprises dyeing a fibrous material with the aid of a dyeing composition containing a dye formed by oxidation, and as another dye, a phenylene dithiourea, one of said dyes being applied first and the other dye being applied later to the fibrous material to be dyed.

8. The process which comprises dyeing a fibrous material with the aid of a dyeing composition containing a member of a group of substances which consists of transformation products of sulfocyanate derivatives of the benzene

80

8

90

91

100

105

110

115

120

125

130

135

140

145

150

- series, the dyeing being conducted in the presence of an oxidizing agent.
9. The process which comprises dyeing a fibrous material with the aid of a dyeing composition containing a member of a group of substances which consists of transformation products of sulfocyanates of the benzene series, the dyeing being conducted in the presence of an oxidizing agent.
10. The process which comprises dyeing a fibrous material with the aid of a dyeing composition containing a phenylene dithiourea, the dyeing being conducted in the presence of an oxidizing agent.
11. The process which comprises dyeing a fibrous material with the aid of a dyeing composition containing a dye formed by oxidation, and as another dye, a member of a group of substances which consists of transformation products of sulfocyanate derivatives of the benzene series, the dyeing being conducted in the presence of an oxidizing agent.
12. The process which comprises dyeing a fibrous material with the aid of a dyeing composition containing a dye formed by oxidation, and as another dye, a member of a group of substances which consists of transformation products of sulfocyanates of the benzene series, the dyeing being conducted in the presence of an oxidizing agent.
13. The process which comprises dyeing a fibrous material with the aid of a dyeing composition containing a dye formed by oxidation, and as another dye, a phenylene dithiourea, the dyeing being conducted in the presence of an oxidizing agent.
14. The process which comprises dyeing a fibrous material with the aid of a dyeing composition containing a member of a group of substances which consists of transformation products of sulfocyanate derivatives of the benzene series, the dyeing being conducted in the presence of an oxidizing agent and an acid.
15. The process which comprises dyeing a fibrous material with the aid of a dyeing composition containing a member of a group of substances which consists of transformation products of sulfocyanates of the benzene series, the dyeing being conducted in the presence of an oxidizing agent and an acid.
16. The process which comprises dyeing a fibrous material with the aid of a dyeing composition containing a phenylene dithiourea, the dyeing being conducted in the presence of an oxidizing agent and an acid.
17. The process which comprises dyeing a fibrous material with the aid of a dyeing composition containing a dye formed by oxidation, and as another dye, a member of a group of substances which consists of transformation products of sulfocyanate derivatives of the benzene series, the dyeing being conducted in the presence of an oxidizing agent and an acid.
18. The process which comprises dyeing a fibrous material with the aid of a dyeing composition containing a dye formed by oxidation, and as another dye, a member of a group of substances which consists of transformation products of sulfocyanates of the benzene series, the dyeing being conducted in the presence of an oxidizing agent and an acid.
19. The process which comprises dyeing a fibrous material with the aid of a dyeing composition containing a member of a group of substances which consists of transformation products of sulfocyanate derivatives of the benzene series, and thereafter removing excess dye, and developing the dye remaining.
20. The process which comprises dyeing a fibrous material with the aid of a dyeing composition containing a phenylene dithiourea, and thereafter removing excess dye, and developing the dye remaining.
- MARTIN BATTEGAY.
- 120
- 110
- 100
- 95
- 90
- 85
- 80
- 75
- 65
- 55
- 45
- 35
- 25
- 130
- 135
- 140
- 145
- 150